

Jan. 11, 1944.

E. VAN DER PYL

2,339,208

FLEXIBLE ABRASIVE PRODUCT

Filed April 4, 1941



EDWARD VANDER PYL

George G. Geary, Attorney

## UNITED STATES PATENT OFFICE

2,339,208

## FLEXIBLE ABRASIVE PRODUCT

Edward Van der Pyl, Holden, Mass., assignor to  
Behr-Manning Corporation, Troy, N. Y., a corporation of Massachusetts

Application April 4, 1941, Serial No. 386,785

3 Claims. (Cl. 51—309)

The invention relates to flexible abrasive products.

One object of the invention is to provide a flexible abrasive product of great tensile strength. Another object of the invention is to provide a flexible abrasive product capable of use at high temperatures, for example, in a furnace. Another object of the invention is to provide an abrasive belt of very rugged construction, which is durable under extreme conditions such as excess of heat or cold, which may be used wet or dry, and which has great tensile strength. Another object of the invention is to provide a flexible abrasive belt utilizing diamonds which are so firmly attached to a durable support that their effective abrading life may be substantially utilized. Other objects will be in part obvious or in part pointed out hereinafter.

The invention accordingly consists in the features of construction, combinations of elements, arrangements of parts, and in the several steps and relation and order of each of said steps to one or more of the others thereof, all as will be illustratively described herein, and the scope of the application of which will be indicated in the following claims.

In the accompanying drawing illustrating one of many possible embodiments of the mechanical features of the invention,

Figure 1 is a view, partly in elevation and partly in section, of apparatus to make the flexible abrasive product, and

Figure 2 is a cross sectional view, on an enlarged scale, of a flexible abrasive product.

I provide a quantity of sheet metal, preferably on a roll, not shown. Cold rolled steel in sheet form is preferred and there are no particular limits to the thickness of the steel. However, it may be noted that for most purposes the steel should be fairly flexible and since the principal utility of the invention is to form abrasive belts, the thickness of the steel will have a relation to the size of the rollers over which the belt runs and a general relation to the character of the abrading operation whether, for example, it involves fast removal of large amounts of stock without any attempt to obtain other than a rough abrading operation or whether, on the other hand, it may involve a fine polishing action. A typical sheet of cold rolled steel is indicated at 10, Figure 1, and this to be coated with abrasive 11 contained in a hopper 12. Within the scope of the present invention the abrasive 11 may be of any suitable type and will

be selected with particular regard to the abrading operation to be performed. For example, for the cutting or polishing of hard carbides, diamond abrasive will preferably be used. For most operations upon tough steel, fused alumina abrasive will be used. For woodworking operations, silicon carbide and in some cases garnet may be used.

The abrasive 11 is to be bonded to the cold rolled steel backing 10 by a metal bond formed from metal powder 13 contained in a hopper 14. Within the scope of the invention, any powders or mixture of powders may be used. However, to obtain resistance to heat, high melting point metals will be utilized, that is, melting at above 250° C. Because they can be obtained in very finely divided form and in a relatively pure state, except for possible oxidation in certain instances, electrolytic metal powders are preferred. For satisfactory results for the bonding of most abrasives, bronzes are desirable which can be formed *in situ* from a mixture of copper and tin powders. If a ductile bronze is wanted, and this may be preferred for certain uses, 5 to 15% of tin, the remainder copper, may be utilized. If a friable copper bond is wanted, and in many situations this will be preferred, above 18% and preferably not more than 35% of tin, the remainder copper may be employed. I may use in certain instances the very hard copper-iron-tin-nickel bond in any of its embodiments described in my U. S. Letters Patent No. 2,238,351. However, any other metals or alloys may be employed within the scope of the invention, such as those disclosed in Milligan Patent 2,077,366, my own prior Patent 2,077,345, and others.

The sheet 10 travels in the direction of the arrow from right to left. It first passes under the hopper 14 where it receives a load of metal 13 which becomes a level deposit 13a extending the entire width of the sheet 10. A spreader guard 15 levels the deposit and spreads it evenly. Any lost off the edges may be recovered and used over again. It is advisable not to try to run the sheet 10 too fast; two or three feet a minute is a satisfactory speed.

The sheet 10 with a layer 13a thereupon then comes under the hopper 12 having an abrasive delivery roll 16 and a guard 17. The roll 16 is rotated slowly to deliver a steady waterfall of abrasive 11a, forming a level superimposed layer of abrasive 11b on top of the layer 13a. Preferably the adjustments of the hopper, guard and delivery roll 16 are such that the layer 11b will only be one abrasive particle thick and the in-

dividual particles should be spaced not too closely together nor, on the other hand, too far apart. The technique of hopper delivery for abrasives is now well understood so I need not further describe the same.

The sheet 10 with layers 13a and 11b now passes between rolls 20 and 21. The roll 20 is preferably a polished steel roll. The roll 21, on the other hand, is preferably a resilient rubber roll. The roll 20 may have trunnions or an arbor 22 mounted in bearings in a pair of frame members 23 of the general shape shown. The lower steel roll 20 is a fixed roll while the upper rubber roll 21 is adjustable in a vertical direction. It has trunnions or an arbor 24 by means of which it is journaled in a pair of vertically movable slides 25 sliding in guideways 26 formed in the frame 23. Screws 27 extending through the top portions of the frame 23 can be used to force downwardly the slides 25 to adjust the pressure.

The action of the rubber roll pressing against the layers 11b and 13a upon the sheet 10 compacts the metal layer 13a but the larger abrasive particles form for themselves temporary pockets in the rubber. Nevertheless the abrasive particles are forced downward until they contact the sheet 10 but their tops protrude above the compacted level of the metal powders. The delivery rates of the metal powders and the grit size of the abrasive 11 should be so chosen that sufficient embedding of the abrasive will occur leaving, however, a substantial volume of the abrasive above the surface. The exact proportion of abrasive embedded and above the surface will vary for different uses and if the known abrasive cloth technique is followed, practical and useful results will be achieved but variations will, of course, suggest themselves for further improvement.

The sheet 10 with compacted layer 13a and abrasive particles 11b embedded therein now passes into a furnace 30 and is there heated to such temperature and for such a period as will cause the metal particles of the compacted layer 13a to fuse, alloy or sinter together to form a strong, rigid and yet somewhat porous structure, at the same time to be strongly and directly bonded to the steel sheet 10. It is preferable to plate the sheet 10 by immersion plating with a coating which may be terne plate, lead, tin, or other suitable soft metal alloy plating. This during the sintering operation in the furnace 30 is absorbed into the metal layer formed by sintering the layer 13a. However, this preliminary plating operation appears to facilitate the union of the metals. But the strength of the union between the steel sheet 10 and the metal layer 13a is far greater than the strength of the soft metal and the heat resistance of the final article is not merely that of the metal plating but is far, far above it.

The sintering should take place in a reducing atmosphere within the furnace 30. Such reducing atmospheres in sintering furnaces are now well known and need not be illustrated and described in much detail herein. A suitable reducing atmosphere consists of flue gas made by incompletely burning natural gas and having from 1% to 7% CO, 7% to 11% CO<sub>2</sub>, 1% to 7% hydrogen, and as little water vapor as is practically possible, for instance, about three-tenths of a pound of water vapor per 1000 cubic feet of the flue gas. The water vapor in the flue gas may be removed by refrigerating the flue gas and thereby condensing the water. The dried flue gas is then passed into the furnace 30 where it is reheated

to the desired sintering temperature, which will be around 600° C. for the copper-tin mixtures mentioned and around 850° C. for the copper-tin-iron-nickel mixtures, for example, equal parts by weight of these metals. In Figure 1 of the drawing, the inlet pipe 31 admits gas to the sintering chamber. An entrance slot 32 for the steel sheet 10 with superimposed layers is only high enough to admit them with slight clearance 10 and the volume of gas entering the furnace 30 is such that there is an outflow at the slot 32. The furnace has an exit slot 33 through which the material being treated passes into a water cooled chamber 34 consisting of water jacketed walls 35 having a water entrance pipe 36 and an outflow pipe 37. The gases from the furnace 30 pass into the cooling chamber 34 and thence out a narrow exit slot 40 for the material which after leaving chamber 34 may be wound upon a 20 drum in a customary manner. The sintering furnace 30 may be heated by suitable electric heating units 41 or in any other desired manner.

The final article illustrated magnified in Figure 2 constitutes an abrasive sheet consisting of a metal backing 10 (which need not necessarily be steel) and abrasive grains 11 secured thereto by a sintered metal bond 13 which is fused to the metal backing 10. For firm embedding of the abrasive particles, more than half of their volume 25 may be embedded, as shown in Figure 2. For long life of the abrasive article, a friable bond 13 can be employed and I have already indicated which are good friable bonds, for example, copper-tin with more than 18% of tin. For a very strong and hard, yet somewhat friable bond quite suitable for diamonds, equal parts of copper, tin, nickel and iron may be used. This bond also adheres very tenaciously to the iron backing and is the preferred embodiment of my invention. Such 30 a bond is highly useful for holding diamonds because it will hold them until they have been completely used up. When the diamonds wear down to the level of the bond, the bond will start to crumble away sufficiently to clear the abrasive 45 for cutting if enough pressure is used. When diamonds are the abrasive, the atmosphere in the furnace 30 should preferably be nitrogen, which is easy to procure, non-poisonous, and which will prevent oxidation of the diamonds.

50 Abrasive belts can be made out of the material of the invention and if they are backed by strong supports and driven by powerful rollers, diamond abrasive belts will cut the hardest of carbides and last through all vicissitudes for years of almost daily use. Abrasive belts constructed according to the present invention, especially if the abrasive is fused alumina, may be run through slots into hot furnaces to do an abrading operation upon white hot metal.

60 It will thus be seen that there has been provided by this invention an article of manufacture and a method in which the various objects hereinabove set forth together with many thoroughly practical advantages are successfully achieved. 65 As various possible embodiments might be made of the mechanical features of the above invention and as the art herein described might be varied in various parts, all without departing from the scope of the invention, it is to be understood that all matter hereinbefore set forth or shown in the accompanying drawing is to be interpreted as illustrative and not in a limiting sense.

I claim:

1. A flexible sheet-like abrasive article comprising abrasive granules embedded in a porous ma-

trix of a sintered metal bond comprising a copper and tin alloy having from 18 to 35 percent of tin, secured on a flexible sheet metal backing, said sintered metal bond being of a porosity permitting the product to flex readily in use.

2. A flexible sheet-like abrasive article comprising abrasive granules embedded in a porous matrix of a sintered metal bond comprising a copper and tin alloy having more than 18 percent of tin, secured on a flexible sheet metal backing, said 10

sintered metal bond being of a porosity permitting the product to flex readily in use.

3. A flexible sheet-like abrasive article comprising abrasive granules supported on a flexible metal sheet by a bond of metal powder, sintered around said abrasive granules, having in its sintered form sufficient porosity to permit flexing of the resultant product.

EDWARD VAN DER PYL.